

1

2,807,527.

## PETROLEUM DISTILLATE COMPOSITIONS CONTAINING FATTY OIL PITCHES

Charles T. Brown and Robert L. Dinsmore, Long Beach, and Wendell F. Deeter, Bellflower, Calif., assignors to Richfield Oil Corporation, a corporation of Delaware

No Drawing. Application February 4, 1954,  
Serial No. 408,287.

5 Claims. (Cl. 44—61)

This invention relates to liquid petroleum hydrocarbons having added thereto small but effective amounts of corrosion inhibiting substances which are residues from refining.

It is well known in the art that rusting or corrosion may occur on steel or iron surfaces in contact with hydrocarbons and water. All types of liquid hydrocarbon products including gasoline, kerosene, thinners, stove oil, diesel oil and residual fuel oil, exhibit this corrosive effect. Corrosion of ferrous metals by leaded gasoline is particularly severe. Water is almost always present in association with hydrocarbons in storage, blending and distribution systems. Water is frequently introduced into petroleum systems with the hydrocarbon itself either in the dissolved or suspended state, and in addition may be intentionally introduced as a bottom seal for a storage tank. The water may even be formed in situ by condensation from the air in a tank due to changes in atmospheric conditions. Further it is common practice to use water as a follower for a particular petroleum stock in a pipe line, to clean and flush lines and tanks with water and to use water in the oil tanks of ships as ballast or for cleaning purposes.

It is obvious that rusting at any point in the manufacturing, distribution or terminal system represents a considerable monetary loss due to extra expense for cleaning and repair of these systems. Under severe conditions of corrosion, it may even be necessary to replace the expensive equipment. Furthermore, rust formed in one part of a fuel system is frequently transported with the fuel to other parts. The rust may plug screens and filters, resulting in inefficient operation or in some cases, complete stoppage. Rust in these systems is particularly detrimental where parts are machined to close tolerances, due to excessive wear caused by the foreign material.

In recent years, in addition to the corrosion problems mentioned above, a new source of greater difficulty has arisen in connection with the use of hydrocarbon solvents for various chemicals which tend to accelerate corrosion. This problem has been particularly troublesome in the case of DDT-hydrocarbon solvent systems. Another corrosion problem has arisen in the wood treating industry where it is customary to use a petroleum solvent for pentachlorophenol. This solution is often subjected to a wide range of temperatures, from atmospheric to 250° F. and to pressures ranging from 15" of mercury vacuum to 150 lbs. per square inch gauge. Further, the presence of water, steam and air is usual. Under these conditions, abnormal corrosion may occur due to the presence of the chlorinated compound and the wide variation in operating conditions. Corrosion in these systems tends to shorten greatly the useful life of the equipment.

In the present invention, liquid petroleum hydrocarbon systems are inhibited against corrosion by having added thereto a rust or corrosion inhibitor which is a fatty acid pitch which is the residue from the refining of a fatty oil, e. g., of animal, vegetable or fish origin. The pitches which are useful are soluble in the liquid petroleum hydro-

2

carbon at least to an extent sufficient to afford the desired inhibiting effect. Mixtures of these pitches are also effective to inhibit rust and corrosion. The fatty acid pitches employed in our invention are in general, viscous, high-boiling substances which are variously described in the art as residues, foots, still-bottoms, break materials, acidulated dewatered soapstocks and pitches.

These pitches are commercially available materials which are produced in conventional fatty oil refining operations. For instance, acidulated dewatered soapstocks are derived from the fatty oil through alkali refining of the oil e. g., see U. S. Patents Nos. 2,100,274 to 2,100,277. The other refining methods affording the desired pitches are acid refining, steam refining or distillation, desliming and degumming methods including hydration and heat treatment and liquid-liquid extraction procedures. All of these methods are well known operations, many of which are described in U. S. Patents, e. g., see Nos. 2,150,732 and 2,201,063. Still-bottoms residues useful in this invention may also be obtained by the splitting of glycerides. Glycerides in raw fatty oils are split with acid-type catalysts and the valuable products removed by vacuum distillation at elevated temperatures. The mixed vegetable oil pitch referred to in Table I below was obtained as a bottoms product in the splitting and vacuum distillation of mixed soya and cottonseed oils.

The vegetable pitches useful in this invention can be obtained as by-products in the processing of cottonseed, flaxseed, soya bean, tung, coconut and other oils of vegetable origin. The marine pitches employed are those obtained as by-products in the processing of whale oil, menhaden oil, cod oil, fish liver oils of any kind and other oils of fish or marine origin. The animal pitches utilized are derived as by-products in the refining of fats and other materials of animal origin. It is the residues from the processing or distillation of these fatty oils, irrespective of their source, which are useful in this invention.

The fatty oil pitches useful in this invention are difficult to define chemically due to differences in source and changes which occur during processing. They can generally be characterized as a mixture of glycerides, unsaponifiables, fatty acids and esters. The pitch may be polymerized to varying degrees depending on processing conditions, i. e., a mixed vegetable and animal pitch may contain approximately 35% glycerides and polymerized material, 25% unsaponifiables and 40% fatty acids and esters. Table I below indicates the approximate composition and boiling range of several pitches which are useful in this invention. The pitches were distilled under vacuum and the values for the distillation temperatures corrected to atmospheric pressure.

TABLE I

| Pitch                               | Tall oil | Acidulated fish oil | Mixed vegetable oil |
|-------------------------------------|----------|---------------------|---------------------|
| Free fatty acids, wt. percent.....  | 67.5     | 55.5                | 45                  |
| Glycerides, wt. percent.....        | 16.5     | 40.0                | 30                  |
| Non-saponifiables, wt. percent..... | 16.0     | 4.5                 | 25                  |
| Distillation, ° F.:                 |          |                     |                     |
| IBP.....                            | 730      | 600                 | 704                 |
| 5%.....                             | 750      | 696                 | 726                 |
| 10%.....                            | 763      | 718                 | 746                 |
| 20%.....                            | 785      | 737                 | 777                 |
| 30%.....                            | 805      | —                   | 800                 |
| 40%.....                            | 820      | 759                 | —                   |

The effectiveness of the fatty oil pitches appears to be due to the fact that these materials preferentially wet metal surfaces, forming a thin, perhaps monomolecular film thereon which is protective against the attack of corrosive materials in contact with the surfaces. The pitches useful in this invention are effective inhibitors for petroleum products such as gasoline, naphthas, thinners, kerosene,

stove oil, diesel oil, lube oils and residual fuel oil, and are useful in any type of manufacturing, distribution or consumer fuel system. Our inhibitors are particularly useful in systems handling light distillates. By light distillates we mean petroleum distillates of a viscosity not exceeding that of gas oil. The inhibiting materials are inexpensive since they are, for the most part, by-products.

The properties of the pitches may vary widely without affecting their value as corrosion inhibitors. Also, pitches from different sources are effective either singly or as a mixture. The table below lists a selection of pitches which are among those effective for the purpose of this invention.

Table II  
Properties of typical pitches

| Pitch source              | Type                     | Sp. gr. at 60° F. | Acid number | Sap. number | Viscosity, S. S. U. V. at 210° F. |
|---------------------------|--------------------------|-------------------|-------------|-------------|-----------------------------------|
| Vegetable.....            | Cottonseed.....          | 1.01              | 38          | 103         | 2,000                             |
| Do.....                   | Soya.....                | .97               | 37          | 139         | 403                               |
| Animal.....               | Swift Ebony Fat #1.....  | .92               | 87          | 183         | 52.2                              |
| Do.....                   | Swift Ebony Fat #40..... | 1.00              | 99          | 161         | 701                               |
| Fish.....                 | Fish.....                | .93               | 109         | 197         | 46.7                              |
| Vegetable and animal..... | Mixed.....               | .982              | 9.4         | 180         | 118                               |
| Fish and animal.....      | O. G. fat.....           | .97               | 39          | 144         | 456                               |

(S. S. U. V.—seconds Saybolt Universal viscosity.)

For the purpose of this invention, the pitch can be used in the form derived from the fatty oil refining procedures, or can be diluted with a solvent, or blended with other materials for facility in handling. For example, a mixed pitch of vegetable and animal origin having a Saybolt Universal viscosity at 210° F. of 118 seconds may be diluted with 2 parts by volume of Stoddard solvent to one part of pitch, thus reducing the viscosity to 87 seconds Saybolt Universal at 60° F. These pitches prevent corrosion by forming a film on the metal surface to be protected thus preventing contact with water, dilute acids and other reactive materials. The pitches are petroleum oil-soluble and can be diluted with any appropriate solvent such as petroleum thinners, aromatics or alcohols.

The effective concentrations of fatty oil pitches for inhibition of corrosion are generally very low. This fact is advantageous because in the concentrations used the materials do not affect the other properties or specifications of the product. In general effective concentrations of pitch range from as little as 1 lb. per 1000 barrels of the liquid petroleum hydrocarbon to be treated to as much as 5 percent by weight. Most of the pitches are dark in color which limits their use in light distillates such as gasoline to 1 lb. to 15 lbs. per 1000 barrels. In lube oils, however, the product color is not so important and concentrations of pitch as high as 5 percent by weight can be employed.

The following specific examples of the use of the inhibiting materials of our invention in various petroleum products will serve to illustrate the invention. The rust ratings referred to in the tables were determined by a modification of ASTM method D-665-52T which is as follows: Gasoline (350 ml.) containing inhibitor is poured into a 400 ml. beaker, a polished steel rod is inserted and the gasoline stirred for a period of 30 minutes. At the end of that time, 50 ml. of hydrocarbon is withdrawn and 30 ml. of water added. Stirring is continued for 3½ hours. At the end of the 3½ hour period, the steel rod is removed and the percentage of rusted surface is estimated. The test is conducted at room temperature in the presence of air and the ratings are made as follows:

4  
TABLE III

| Rating:  | Percent rust |
|----------|--------------|
| A.....   | None.        |
| B++..... | Trace.       |
| B+.....  | Less than 5. |
| B.....   | 5-25.        |
| C.....   | 25-50.       |
| D.....   | 50-75.       |
| E.....   | 75-100.      |

10 The effect of pitch concentration on the rust rating of a leaded ethyl gasoline is shown in the table below. The pitch used was a mixed animal-vegetable pitch having a saponification number of 180.

TABLE IV

| Concentration lbs./M bbls.: | Rust rating |
|-----------------------------|-------------|
| 0.....                      | E           |
| 1.....                      | B+          |
| 3.....                      | B++         |
| 5.....                      | B++         |
| 15.....                     | B++         |

45 The effectiveness of corrosion inhibitors of this invention does not depend on the source of the residues or pitches used. This fact is illustrated by Table V below which shows the rust rating obtained by using pitches from various sources in a leaded gasoline at a concentration of 2 lbs. per 1000 barrels.

TABLE V

| Pitch:                                       | Rust rating |
|----------------------------------------------|-------------|
| None.....                                    | E           |
| Fish.....                                    | B++         |
| Vegetable (cottonseed).....                  | B++         |
| Vegetable (soya).....                        | B           |
| Animal (Ebony fat #1).....                   | B           |
| Animal (Ebony fat #40).....                  | B+          |
| Mixed vegetable & animal (140 Sap. No.)..... | B++         |
| Mixed vegetable & animal (180 Sap. No.)..... | B++         |
| Mixed fish and animal.....                   | B++         |
| Vegetable (Tall oil).....                    | B++         |

50 Static tests have also been used to demonstrate the effectiveness of pitch as a corrosion inhibitor in leaded gasoline in low concentration. A mixed animal-vegetable pitch having a saponification number of 180, produced the results shown in Table VI below.

TABLE VI

| Concentration lbs./M bbls.: | Rust rating |
|-----------------------------|-------------|
| 0.....                      | E           |
| 1.....                      | C           |
| 2½.....                     | B           |
| 5.....                      | B++         |

55 The static test is run using a piece of ASTM grade 1010 steel, 1½" x 5" x 1½", which has been sanded to re-

move all traces of rust and corrosion and then degreased by washing with benzene and acetone, followed by heating at 230-250° F. for thirty minutes. The strip is placed in a 6-oz. bottle containing 150 ml. of the product to be tested and shaken for 30 minutes. Fifteen ml. of distilled water is added and shaking continued for 10 minutes more. The bottle is placed in an inclined position to prevent the end of the steel strip from remaining in direct contact with the main body of water. Before placing in the inclined position, the bottle is generally 10 shaken to suspend water and leave droplets on the top surface of the strip. The bottle is left undisturbed for 24 hours, then is gently shaken and turned over with the other side of the metal strip facing upwards. After another 24 hours, the steel strip is rated according to the 15 scale employed for the modified ASTM method D-665-52T tests.

The pitches of this invention in addition to being effective corrosion inhibitors are also stabilizing agents for tetraethyl lead in gasoline against the action of sunlight. It is common knowledge that commercial gasoline now on the market containing tetraethyl lead becomes cloudy when exposed to direct sunlight, due to the decomposition of the lead compound. When modern gasoline pumps are used, the decomposition of tetraethyl lead is not particularly troublesome because the gasoline is not exposed to direct sunlight. This is not true, however, in old style gasoline pumps which frequently have a 10-gallon glass bowl which is exposed to sunlight. When gasoline is allowed to stand for any length of time in the old style pumps, a cloudy precipitate is likely to form. The stabilizing effect of our inhibiting pitches has been shown by exposing samples of leaded gasoline with and without the inhibitor in clear glass bottles to direct sunlight. The gasoline tested contained approximately 2 cc. of tetraethyl lead per gallon. It was noted that the first decomposition of lead in the uninhibited sample occurred after 3½ hours, the initial decomposition of lead compound in the sample inhibited with a vegetable-animal pitch in a concentration equivalent to 2 lbs. of pitch per 1000 barrels was 13½ hours. Still bottoms from the distillation of soya beam oil and cottonseed oil were found to exhibit similar properties of stabilization for tetraethyl lead in gasoline.

A further example of the results obtained by the corrosion inhibitor of this invention is as follows: The test consisted of incorporating a mixed vegetable oil pitch at a concentration of 5 lbs. per 1000 barrels in a stove oil with a neat rust rating of "E." The rust rating of the inhibited sample was B++.

An example of the effectiveness as corrosion inhibitors of the pitches of this invention when used in jet fuel is illustrated by the results shown in Table VII.

TABLE VII

| Pitch                                 | Concentration, Lb./M bbls. | Rust rating |
|---------------------------------------|----------------------------|-------------|
| None                                  | 0                          | D           |
| Mixed animal-vegetable (140 Sap. No.) | 2½                         | A           |
| Do                                    | 5                          | A           |
| Do                                    | 10                         | A           |
| Mixed animal-vegetable (180 Sap. No.) | 2½                         | A           |
| Do                                    | 5                          | A           |

It is one of the advantages of this invention that the amounts of inhibitors necessary for effective protection against corrosion are so small that the essential specifications of the petroleum products inhibited are not changed. This fact is illustrated by Table VIII below which records the data from a series of tests on samples of leaded gasoline with and without inhibitors to show the difference in physical properties.

6  
TABLE VIII

| Mixed animal-vegetable oil pitch (140 Sap. No.) | Lb./M bbls. |        |
|-------------------------------------------------|-------------|--------|
|                                                 | 0           | 2      |
| Oxygen stability, hours                         | 26          | 27     |
| Gums:                                           |             |        |
| ASTM                                            | 1           | 1      |
| 4 hour                                          | 1.6         | 1.8    |
| Cu dish                                         | 3           | 3      |
| Color                                           | Copper      | Copper |
| Appearance                                      | Bright      | Bright |
| Rust rating                                     | E           | B++    |

The pitches of this invention are also effective as corrosion inhibitors in lube products at concentrations as low as .01% to as much as 5% by weight. Tests made with a western refined turbine oil gave the results shown in Table IX below. The ratings in Table IX were determined by ASTM method D-665-52T, which is a tentative method for determining the rust-preventing characteristics of steam turbine oil in the presence of water. The procedure is the same as the modified method described above for testing gasoline, except that the sample is run in a controlled temperature bath at 140° F. for a period of 24 hours after the addition of water. A passing rating requires that there be no visible rust spots on a steel test specimen.

TABLE IX

| Pitch source    | Type      | Concentration, w.t. percent | Rust rating |
|-----------------|-----------|-----------------------------|-------------|
| Vegetable       | Soya      | 0.2                         | Passes.     |
| Do              | do        | 0.5                         | Do.         |
| Do              | Tall oil  | 0.2                         | Do.         |
| Fish and animal | O. G. fat | 0.2                         | Do.         |
| Do              | do        | 0.5                         | Do.         |

Certain pitches due to their dark color may not in certain instances be suitable for use at the required concentrations in certain products. There are, however, other pitches such as tall oil pitch which are light enough in color to be useful at the required concentrations in these special products.

It has been found that concentrations as low as .01% by weight of the corrosion inhibitors of this invention frequently provide as much as 98% corrosion protection when added to special solvents used as carriers for other chemicals; however, it is occasionally necessary to use concentrations as high as 1% of corrosion inhibitor for satisfactory results. As a specific example of this application of our invention, a small quantity of inhibitor was added to 200 cc. of a petroleum hydrocarbon solvent containing 5% by weight of pentachlorophenol. This mixture was transferred to an oxygen stability tube and 2% water added. A polished steel strip 1" x 10" and a block of fir, ½" x ¾" x 3" were then inserted into the tube. The tube was placed in the bomb of a conventional oxygen stability apparatus and kept under 100 lbs. of oxygen pressure at a temperature of 212° F. for three hours. The bomb was then depressured and the tube removed and allowed to stand for 16 hours. The steel strip was inspected for rusting and the results reported in terms of the rust-rating scale described above. The results are shown in Table X below.

TABLE X

| Mixed animal-vegetable pitch (140 Sap. No.) | Rust rating |             |             |
|---------------------------------------------|-------------|-------------|-------------|
|                                             | Oil phase   | Water phase | Vapor phase |
| 0 wt. percent                               | E           | C           | B           |
| .025 wt. percent                            | B+          | B+          | B           |
| .05 wt. percent                             | B+          | B+          | B++         |
| .1 wt. percent                              | B++         |             |             |

In practice, the additives of this invention are usually present in such small amounts that their presence is difficult to detect in petroleum products. It has been found that corrosion protection afforded by the additives of this invention is due, not only to one, but to many components of the pitch. A sample of mixed animal-vegetable pitch, saponification No. 180, was extracted with acetone and both the extract and the raffinate phases tested in a sample of leaded gasoline having a neat rust rating of "E." Both phases of the pitch gave a rating of B++ when used at a concentration of two lbs. per 1000 bbls. of gasoline.

We claim:

1. A composition consisting essentially of a light petroleum distillate having incorporated therein a soluble fatty oil pitch in an amount effective as a corrosion inhibitor, said amount being from 1 to 15 pounds per thousand barrels of said distillate. 15
2. The composition of claim 1 wherein said distillate is gasoline. 20
3. The composition of claim 1 wherein said distillate is a leaded gasoline.
4. A composition consisting essentially of a light

petroleum distillate having incorporated therein a tall oil pitch in an amount effective to inhibit corrosion, said amount being from 1 to 15 pounds per thousand barrels of said distillate.

5. A composition consisting essentially of a light petroleum distillate containing tetraethyl lead and having incorporated therein a soluble fatty oil pitch in an amount effective to inhibit corrosion and to stabilize tetraethyl lead, said amount being from 1 to 15 pounds per thousand barrels of said distillate.

References Cited in the file of this patent

UNITED STATES PATENTS

|           |                   |                |
|-----------|-------------------|----------------|
| 2,014,235 | Lowry             | Sept. 10, 1935 |
| 2,339,796 | Musher            | Jan. 25, 1944  |
| 2,596,065 | Brabets           | May 6, 1952    |
| 2,668,138 | Walker et al.     | Feb. 2, 1954   |
| 2,671,761 | Kalinowski et al. | Mar. 9, 1954   |
| 2,686,713 | White et al.      | Aug. 17, 1954  |

OTHER REFERENCES

"Industrial and Engineering Chemistry," vol. 40, pages 2338-2347, December 1948.